

# United States Patent [19]

Slowski et al.

[11] Patent Number: 5,044,066

[45] Date of Patent: Sep. 3, 1991

## [54] ELECTRODE RECEPTACLE

[75] Inventors: Wasył Slowski; Darrel Slowski, both of Islington; David Slowski, Mississauga, all of Canada

[73] Assignee: Williams Sign Supplies Ltd., Mississauga, Canada

[21] Appl. No.: 544,950

[22] Filed: Aug. 23, 1990

### Related U.S. Application Data

[63] Continuation of Ser. No. 137,672, Dec. 24, 1987, abandoned.

[51] Int. Cl. 5 H01B 19/00

[52] U.S. Cl. 29/631; 29/173; 439/244; 439/934

[58] Field of Search 439/226-244, 439/736, 934; 72/13, 69, 342.1, 342.5, 342.8; 29/173, 631

## [56] References Cited

### U.S. PATENT DOCUMENTS

- |                                  |         |
|----------------------------------|---------|
| 3,539,969 11/1970 Johnson et al. | 439/231 |
| 3,711,917 1/1973 Baumgras        | 29/173  |
| 3,778,877 12/1973 Walker         | 29/173  |
| 4,229,780 10/1980 Nelson         | 439/242 |
| 4,387,947 6/1983 Lostomo et al.  | 439/840 |
| 4,444,446 4/1984 Hageman         | 439/230 |
| 4,460,226 7/1984 Hageman         | 439/226 |

4,620,763 11/1986 Mochida 439/275

Primary Examiner—David L. Pirlot

Attorney, Agent, or Firm—Eugene J. A. Gierczak

## [57] ABSTRACT

In a method of producing electrode receptacle assemblies for resisting sudden heat increases comprising the steps of selecting carbonate resin plastic having a density of 1.2 mg/m<sup>3</sup>, melt flow rate of 9 to about 12 g/10 m at 300 degrees Centigrade and 1,200 g load, and a tensile stress at yield of 63 MPa, a tensile stress at break of 68 MPa, a deflection temperature under load at 1.8 MPa of 133 degrees Centigrade and a dielectric stress of greater than 16 KV/mm; extruding the selected carbonate resin plastic to form the electrical receptacle with at least one hollow cylindrical section having two open ends; spinning a piece of PH bronze into a coil; subjecting said PH bronze coil to a temperature of 400 degrees Centigrade for a period of one half hour; air cooling said PH bronze coil to room temperature; introducing high tension wire means through the one open end of said electrode receptacle and connecting same to the coil; locating the coil interiorly of the electrode receptacle at the one open end; introducing light means at the other open end for electrical connection to the coil and the high tension wire means to assemble the electrode receptacle capable of resisting sudden heat increases within said hollow cylindrical section.

6 Claims, 1 Drawing Sheet





## ELECTRODE RECEPTACLE

This is a continuation of application Ser. No. 07/137,672, filed Dec. 24, 1987 now abandoned.

## FIELD OF INVENTION

This invention relates to electrode receptacles or sockets, and in particular relates to neon receptacles comprised of polycarbon plastic, and also relates to a 10 stress relieved spring associated therewith.

## BACKGROUND TO THE INVENTION

Displayed tubes such as neon signs are usually mounted in a display or sign housing supported on the exterior wall of a building and electrical connections are made through a conduit to a high tension wire extending through the conduit from the housing through the wall to the interior side of the wall to a power source. Electrodes are mounted on the opposite ends of a gas 15 filled tube or neon sign and are adapted for connection to the ends of the high tension wires.

Since relatively high voltages in the vicinity of 7500 volts are utilized to excite the neon tubes an electrode receptacle or socket has been developed so as to avoid the manual engagement of the electrodes of the neon signs to the high tension wires.

Such electrode sockets usually comprise a cylindrical receptacle or socket which is adapted to be mounted within a cylindrical metal housing and which is adapted for mounting through the building wall on which the sign is mounted. One end of the receptacle which is mounted within the building wall includes a compression spring attached to an electrical contact which is connected to the high tension wires, while the other end of the electrode receptacle includes an opening to telescopingly receive the electrodes at the end of the neon tube for contact with the compression spring, electrical contacts and high tension wire at the other end of the electrode socket. Once the neon tube is inserted into the receptacle the compression spring is compressed so as to effect a good electrical contact. In this way, the electrical connection to the tube is made within the interior of the electrode socket away from the manual engagement and the connection is made automatically upon insertion of the neon tube into the electrode receptacle.

The electrode receptacles have heretofore been made from materials having high dielectric characteristics as insulators such as glass or porcelain.

For example, U.S. Pat. No. 1,872,593 discloses an electrode housing made of porcelain. U.S. Pat. No. 1,890,680 teaches a socket which consists of tubular glass or porcelain. Moreover U.S. Pat. No. 2,046,960 55 teaches the use of an insulator made of Pyrex type or Boro-Silicate glass composition. Finally, U.S. Pat. Nos. 2,486,497 and 2,561,954 show the use of a receptacle or socket made of glass.

The utilization of such fragile material as glass or porcelain in the manufacture of electrode receptacles cause problems in the installation of same as glass or porcelain cracks if mishandled or over tightened. Furthermore, glass and porcelain crack due to changing weather conditions, temperature changes caused by seasonal changes as well as sudden surges of high voltages which vaporize water that tends to collect in the electrical receptacles.

When the glass or porcelain receptacles present cracks, the high electrical voltages leak out or "arc" 5 outwardly through the crack thereby creating a potentially hazardous.

Furthermore, when a building which contains neon tubes is under fire, the severe temperature of the fire as well as the structural damage caused thereby frequently causes the glass or porcelain receptacles to break thereby exposing the high voltages and further creating a dangerous condition.

Also the compression springs used heretofore have a tendency to lose their compressibility or resiliency as a result of the turning on and off of neon tubes over an extended period of time. When neon tubes are turned on 20 or excited by the application of the relatively high voltages the compression spring has a tendency to heat up and expand; and the compression spring has a tendency to cool off or contract when the neon tubes are turned off. Over time this repetitive expansion and contraction 25 of the compression spring causes the spring to lose its resiliency or compressibility to such an extent that the spring may no longer contact the end of the neon tube 30 since the neon tube is anchored to the building wall. 35 When this condition is reached the high electrical voltages arc between the space between the compression 40 spring and end of the neon tube, causing the neon tube 45 to flicker on and off and the neon tube eventually fails.

Furthermore the resulting arcing becomes a potential 50 hazard.

## OBJECTS OF THE INVENTION

It is an object of this invention to provide an electrode receptacle which exhibits improved strength characteristics against cracking.

It is a further object of this invention to provide an improved electrode receptacle which is less costly to produce than those of the prior art.

It is a further object of this invention to provide a more efficient compression spring utilized in the electrode receptacle.

## FEATURES OF THE INVENTION

It is an aspect of this invention to provide a method of producing electrode receptacle assemblies for resisting sudden heat increases comprising of: selecting carbonate resin plastic having a density of 1.2 mg/m<sup>3</sup>, melt flow rate of 9 to about 12 g/10 m at 300 degrees centigrade and 1,200 g load, and a tensile stress at yield of 63 MPa, tensile stress at break of 68 MPa, a deflection temperature under load at 1.8 MPa of 133 degrees centigrade and a dielectric stress of greater than 16 KV/mm; extruding the selected carbonate resin plastic to form the electrical receptacle with at least one hollow cylindrical section having two open ends; spinning a piece of PH bronze into a coil; subjecting said PH bronze coil to a temperature of 400 degrees centigrade for a period of one half hour; air cooling said PH bronze coil to room temperature; introducing high tension wire through the one open end of the electrode receptacle and connecting same to said coil; locating the coil interiorally of the electrode receptacle at the one open end; introducing light at the other end for electrical connection to the coil and the high tension wire to assemble the electrode receptacle capable of resisting sudden heat increases within the hollow cylindrical section.

## DRAWINGS

These and other objects and features are illustrated and described in the following specification to be read in conjunction with the sheets of drawings in which:

FIG. 1 is a cross sectional view of said electrode receptacle.

FIG. 2 is a bottom view of said electrode receptacle.

FIG. 3 is a partial side view of said electrode receptacle.

## DESCRIPTION OF THE INVENTION

Identical parts have been given identical numbers throughout the figures.

The electrode receptacle is generally illustrated as 10 in FIG. 1.

The electrode receptacle 10 comprises generally two hollow cylindrical sections 12 and 14 integrally connected to one another. Hollow cylindrical section 12 is larger in diameter than cylindrical section 14, and is adapted to receive at one end thereof the ends of a neon tube in a manner to be described more fully herein.

Hollow cylindrical section 14 is adapted to receive the high tension wire 16 through conduit 17. Hollow cylindrical section 14 contains three rigidifying ribs 15 as best illustrated in FIG. 2.

The electrode receptacle 10 is adapted to be received by a metal sleeve 18 which is adapted to be mounted on the exterior of a building wall 20 as illustrated in FIG. 1. Alternatively, the metal sleeve 18 may be mounted in a sign housing (not shown) in a manner well known to those skilled in the art. The metal sleeve 18 is grounded by wire 19.

The high tension wire 16 passes through hollow cylindrical section 14 and is connected to plate 22. Plate 22 is in electrical contact with compression spring 24.

FIG. 1 illustrates one end of neon tube 30 which contains an electrode 32 at one end thereof and is adapted to be telescoped into one end of the electrical receptacle 10 so as to make contact with compression spring 24, plate 22, and high tension wire 16.

The other end of neon tube 30 (not shown) is adapted to be telescoped within another electrode receptacle (not shown) identical to the one illustrated in FIG. 1.

Once the neon tube 30 is inserted as described, neon tube 30 is fixedly retained or anchored to the building wall 20 by means of a support and tie wires 40.

The electrode receptacle 10 is made of a plastic made from polycarbonate resins. The polycarbonate plastic utilized in the present invention is flame retardant such as identified by the trademark Merlon 6455 having the following physical properties:

|                                              |                       |
|----------------------------------------------|-----------------------|
| Density                                      | 1.2 Mg/m <sup>3</sup> |
| Melt Flow Rate<br>(300° C. - 1200 g Load)    | 9-12 g/10 m           |
| Tensile Stress at Yield                      | 63 MPa                |
| Tensile Stress at Break                      | 68 MPa                |
| Deflection Temperature Under Load at 1.8 MPa | 133° C.               |
| Dielectric Strength                          | Greater Than 16 KV/mm |

It has been found that by utilizing polycarbonate plastics in the manufacture of electrode receptacles, the chances of cracking electrode receptacle 10 is minimized as polycarbonate plastic is not as fragile as glass or porcelain. Accordingly, less arcing problems occur with the utilization of electrode receptacles made from polycarbonate plastics than with glass or porcelain.

Furthermore, it has been found that electrode receptacles made from polycarbonate plastics and specifically Merlon 6455 resist the formation of cracking which may occur in glass and porcelain when very high voltages are turned on particularly when rain water or water droplets accumulate in the electrode receptacle. Under such conditions, the sudden surge of a very high voltage "frys" the water within the electrode receptacle to very high temperatures so as to vaporize same. The almost instantaneous temperature differential which occurs in the water collected in the electrode receptacles tends to enhance the formation of cracks in the electrode receptacles made from glass or porcelain. It has been found that electrode receptacles 10 made from polycarbonate resist the formation of cracks due to the sudden surge of high voltages to the collected water.

Moreover, it has been found that the polycarbonate resins will melt over compression spring 24, plate 22 and high tension wire 16 when exposed to elevated temperatures such as during a fire so as to create an insulating coating over same, thereby minimizing the exposure of "live wires" having a very high voltage. Electrode receptacles made of glass or porcelain tend to crack under such conditions thereby enhancing arcing and exposing an electrical hazard.

The electrical receptacles made from polycarbonate plastics may be produced in one piece by plastic extrusion methods in a highly mechanized manner so as to bring down the cost of manufacture. For example, electrode receptacles made from polycarbonate plastics may be manufactured for approximately one-third to one-quarter the cost of electrical receptacles made from glass or porcelain.

Electrode receptacles made from glass as illustrated in FIG. 1 are typically made in two separate pieces namely cylindrical sections 12 and 14 which are melted and fused together in the area of common contact marked 13. This procedure is relatively costly and time

consuming and the melted zone 13 presents an area of weakness. Electrode receptacles made from polycarbon resins on the other hand may be made in one piece by extrusion means in a fast and efficient manner.

Electrode receptacles made from heat resistant glass have a tendency to crack when subjected to a thermal shock test by exposing same to a temperature differential between 0° C. and 100° C. repetitively five times. Electrode receptacles made of Pyrex glass usually withstand such thermal shock tests although Pyrex glass is relatively expensive relative to electrode receptacles made from polycarbon plastics. It has been found that electrode receptacles made of Herlon 6455 successfully pass thermal shock tests between -42° C. to 100° C.

As described earlier the compression springs which have been used before have a tendency to loss their resiliency and eventually no longer contact electrode 32 of neon tube 30 after prolonged usage as illustrated by the hidden lines in FIG. 1. (The gap between the compression spring represented by the hidden lines in FIG. 1 at the electrode 32 has been exaggerated for illustration purposes.)

It has been found that this condition may be delayed by using heat tempered compression springs. More specifically it has been found that if a straight piece of PH Bronze also known as Foster Bronze is spun into the shape of the coil and then heat tempered at 400° C. for  $\frac{1}{2}$  hour and then air cooled to room temperature the resulting compression spring exhibits superior compression characteristics even after prolonged exposure to temperature changes between -42° C. and 450° C. resulting in a longer effective life of the compression spring and the neon tube since the compression spring contacts the electrode 32 for a longer period of time than compression springs which are not heat tempered. This delays the destructive action of the arcing between the compression spring 24 and electrode 32.

It has been found that electrode receptacle made of Herlon 6455 having a thickness of 3/16 inch walls are suitable.

Although the preferred embodiments, as well as the operation and use have been specifically described in relation to the drawings, it should be understood that variations in the preferred embodiments could easily be achieved by a skilled man in a trade without departing from the spirit of the invention. Accordingly, the invention should not be understood to be limited to the exact form revealed in the drawings.

The embodiments of the invention in which an exclusive property or privilege is claimed are defined as follows:

5 1. In a method of producing electrode receptacle assemblies for resisting sudden heat increases comprising the steps of:

- (a) selecting carbonate resin plastic having a density of 1.2 mg/m<sup>3</sup>, melt flow rate of 9 to about 12 g/10 m at 300 degrees centigrade and 1,200 g load, and a tensile stress at yield of 63 MPa, a tensile stress at break of 68 MPa, a deflection temperature under load at 1.8 MPa of 133 degrees centigrade and a dielectric stress of greater than 16 KV/mm;
- (b) extruding said selected carbonate resin plastic to form said electrical receptacle with at least one hollow cylindrical section having two open ends;
- (c) spinning a piece of PH bronze into a coil;
- (d) subjecting said PH bronze coil to a temperature of 400 degrees centigrade for a period of one half hour;
- (e) air cooling said PH bronze coil to room temperature;
- (f) introducing high tension wire means through said one open end of said electrode receptacle and connecting same to said coil;
- (g) locating said coil interiorly of said electrode receptacle at said one open end;
- (h) introducing light means at said other open end for electrical connection to said coil and said high tension wire means to assemble said electrode receptacle capable of resisting sudden heat increases within said hollow cylindrical section.

2. In a method of producing electrode receptacles as claimed in claim 1 wherein said electrode receptacles have walls of approximately 3/16th of an inch.

3. In a method of producing electrode receptacles as claimed in claim 1 wherein said electrode receptacle is extruded so as to present two hollow cylindrical sections integrally connected together.

4. In a method of producing electrode receptacles as claimed in claim 3 wherein one of said hollow cylindrical sections is larger than said other hollow cylindrical section.

5. In a method of producing electrode receptacles as claimed in claim 4 wherein said coil is placed in said smaller cylindrical section.

6. In a method of producing electrode receptacles as claimed in claim 5 wherein a high tension wire is connected interiorly of said electrode receptacle to said coil in said smaller cylindrical section.

\* \* \* \* \*